

## 1

3,285,736

## POWDER METALLURGICAL ALLOY

Walter K. Brinn, Euclid, and Ronald L. Barto, Wickliffe, Ohio, assignors to General Electric Company, a corporation of New York  
 No Drawing. Filed Aug. 27, 1964, Ser. No. 392,649  
 3 Claims. (Cl. 75—122.5)

This invention relates to powder-metallurgical molybdenum-base alloys, and, more particularly, to such alloys strengthened both by solid solution and dispersion hardening so as to provide an alloy having high strength at elevated temperatures and good workability at room temperature.

In satisfying requirements for refractory metal alloys, arc-casting is often used to produce complex, multi-phase alloys that can be heat-treated in combination with deformation processing to give materials having good adaptability, the structure and properties of which can be altered during manufacture to meet the end requirements. Alloys produced by powder metallurgy, on the other hand, have in the past been considered to be much less amenable to thermal and mechanical treatments to vary their properties. Problems of purity and difficulties in obtaining homogeneity in alloys produced from powder, rather than by melting, limited the availability of powder-metallurgical refractory metal alloys except for specialized purposes such as filament and support wire for lamps and electronic tubes.

Conversely, the costs involved in producing arc-cast refractory metal alloys are generally several times those necessary for the production of refractory metal alloys by powder-metallurgical methods, provided useful powder alloys could be designed and produced in a homogeneous, stable condition free from deleterious effects of impurities. It would be especially desirable from a cost standpoint to be able to provide reliable and reproducible powder-metallurgical alloys based on molybdenum and hardened by a combination of solid solution strengthening and dispersion hardening that would be workable at or near room temperature and have satisfactory ductility at room temperature and sufficient strength at elevated temperatures.

Many of the commercial arc-cast refractory metal alloys contain alloying additions such as zirconium and titanium which may form compounds such as carbides and oxides that are susceptible to reversible dissolution and precipitation in the matrix phase, thus allowing the titanium or zirconium additive to serve either as a solid solution strengthener or as a dispersoid or both in combination. It is readily apparent that thermal and mechanical treatments for such alloys cannot be consistently controlled to account merely for stress-relief and recrystallization, but also must account for partial or complete precipitation, dissolution, agglomeration and morphology of the precipitate. This is in strong contrast to the stability of properties that theoretically could be made available in insoluble dispersoid powder-metallurgical alloys. However, useful powder-metallurgical alloys of molybdenum have not heretofore been available having sufficiently desirable combinations of properties to satisfy certain of the demands of industry.

Accordingly, it is an object of the present invention to provide powder-metallurgical molybdenum-base alloys strengthened by both solid solution and dispersion hardening that have greatly improved strength at elevated temperatures and are workable at room temperature.

It is another object of the present invention to provide such alloys that are equivalent or superior in their properties to current commercial arc-cast refractory metal alloys.

## 2

Briefly stated, the present invention accomplishes the above-mentioned objects and others by providing a powder-metallurgical molybdenum-base alloy consisting essentially of, by weight, about 0.1-1% thoria ( $\text{ThO}_2$ ) and about 5-30% tungsten, the balance being molybdenum. Among the preferred and optimum ranges of compositions of molybdenum-base alloys within the invention are 0.1-0.25%  $\text{ThO}_2$  with 15-25% tungsten, and about 0.2%  $\text{ThO}_2$  with about 20% tungsten.

Alloys of the invention are made with conventional powder-metallurgical processing equipment. The desired quantities of tungsten, molybdenum and thoria, powders can be blended together in a V or "twin shell" blender with an intensifier for about twenty minutes with the approximate particle sizes for the constituents being given in Fisher number as: molybdenum—2.8, tungsten—1.3, and thoria—0.7. The blended powders may be packed in rubber containers having a rectangular cross section, sealed and pressed hydrostatically at a pressure of about 35,000 pounds per square inch. The green compacts, which are self-supporting after compaction, can then be sintered in a hydrogen furnace for about 15 hours at about 1850° C.

As is well known in the art, many types of processes can be used to convert such sintered billet into wrought products such as sheet or bar. As an example of one process for the production of sheet from sintered billet, the billet can be heated in a hydrogen atmosphere to 1200° C. and then rolled in drafts of preferably 10-20% per pass to a total reduction of about 50% with reheating as necessary to keep the metal between 900 and 1200° C. The metal is then recrystallized and rolled to finish-gage sheet, preferably between 900 and 1200° C. at 10-20% per pass, followed by a stress-relief anneal. The amount of reduction per pass may depend on the capacity of the rolling mill.

Stress-relief annealing of the wrought product can be accomplished by heating in the temperature range of 900° C. to 1200° C. for times of about one hour. The wrought material can be recrystallized by heating in a temperature range of 1100° C. to 1400° C. for about one hour.

Table I shows the superiority of an alloy of the invention over unalloyed powder-metallurgical molybdenum in terms of increased recrystallization temperature and finer grain size as recrystallized. All material was warm rolled with a 92% reduction in thickness. Start and completion of recrystallization were determined for times of ten minutes at temperature in a hydrogen atmosphere furnace.

TABLE I  
 [Recrystallization characteristics]

| 55 | Material                          | Recrystallization<br>(° F.) |          | Grain Size<br>(grains/mm. <sup>2</sup> ) |
|----|-----------------------------------|-----------------------------|----------|------------------------------------------|
|    |                                   | Start                       | Complete |                                          |
| 60 | Unalloyed Mo.....                 | 1,740                       | 2,010    | 4,000-4,500                              |
|    | Mo-20W-0.2 ThO <sub>2</sub> ..... | 2,190                       | 2,600    | 8,000-10,000                             |

Table II below gives typical room temperature (about 78° F.) properties of an alloy of the invention containing about 20% tungsten and 0.2% thoria, balance molybdenum rolled to three different thicknesses of sheet. In each table, K s.i. stands for thousands of pounds per square inch; the strain rate used in testing was 0.005 inch per inch per minute to the 0.6% offset yield point and then 0.05 inch per inch per minute to failure. The longitudinal direction (long.) is parallel to the rolling direc-

tion, and the transverse direction (trans.) is perpendicular to the rolling direction but in the plane of the sheet. The Tinus-Olsen cup depth is a measure of the formability of the sheet, with a greater depth indicating greater workability.

melting and recrystallization temperatures over unalloyed molybdenum also have been achieved in these powder-metallurgical alloys without losing the type of low temperature ductility and workability characteristic of the unalloyed metal.

TABLE II

[Typical room temperature properties of Mo-20W-0.2 ThO<sub>2</sub>]

| Thickness (inches) | Direction  | Tensile Strength (K s.i.) | 0.2% Yield Strength (K s.i.) | Percent Elongation in 1 inch | Tinus-Olsen cup depth (inches) |
|--------------------|------------|---------------------------|------------------------------|------------------------------|--------------------------------|
| 0.010.....         | Long.....  | 133                       | 109.5                        | 7.5                          | 0.198                          |
| 0.010.....         | Trans..... | 134                       | 114.5                        | 6.5                          | 0.198                          |
| 0.015.....         | Long.....  | 127                       | 105                          | 13.0                         | 0.224                          |
| 0.015.....         | Trans..... | 131                       | 112.5                        | 7.0                          | 0.242                          |
| 0.030.....         | Long.....  | 127.5                     | 105                          | 13.0                         | 0.256                          |
| 0.030.....         | Trans..... | 135                       | 114                          | 11.5                         | 0.256                          |

Table III below presents a comparison of the properties of an alloy of the invention containing about 20% tungsten, 0.2% thoria, balance molybdenum, unalloyed molybdenum produced by powder-metallurgical means and arc-cast molybdenum containing about 0.5% titanium, all in the form of 40 mil thick sheet. SR means stress-relieved 1 hour at 1850° F. for the 20W-0.2% ThO<sub>2</sub> alloy and Mo-0.5 Ti, while the pure molybdenum was stress-relieved at 1750° F. for 1 hour.

It is intended that this invention be interpreted as broadly as the true scope and spirit of the appended claims.

What we claim as new and desire to secure by Letters Patent of the United States is:

1. A molybdenum-base powder-metallurgical alloy workable at room temperature consisting essentially of by weight from about 0.1% to about 1% ThO<sub>2</sub>, from about 5% to about 30% tungsten, and the balance molybdenum,

TABLE III  
[Comparative properties]

| Alloy                       | Condition | Temper-ature (° F.) | Tensile Strength (K s.i.) | 0.2% Yield Strength (K s.i.) | Percent Elongation in 1 inch |
|-----------------------------|-----------|---------------------|---------------------------|------------------------------|------------------------------|
| Mo-20W-0.2 ThO <sub>2</sub> | SR.....   | 78                  | 130                       | 110.0                        | 20                           |
|                             | SR.....   | 1,800               | 69                        | 45.0                         | 10                           |
|                             | SR.....   | 2,200               | 38                        | 22.5                         | 30                           |
|                             | RX.....   | 2,500               | 22                        | 8                            | 60                           |
|                             | RX.....   | 2,600               | 17.5                      | 9.3                          | 19                           |
|                             | RX.....   | 2,800               | 13.5                      | 5.0                          | 34                           |
|                             | RX.....   | 3,000               | 10.5                      | 4.5                          | 44                           |
|                             | RX.....   | 3,200               | 7                         | 2.5                          | —                            |
| Unalloyed Mo.....           | SR.....   | 78                  | 110                       | 92                           | 20                           |
|                             | SR.....   | 1,800               | 51                        | —                            | —                            |
|                             | SR.....   | 2,200               | 16.5                      | —                            | —                            |
|                             | SR.....   | 2,400               | 11.5                      | —                            | —                            |
|                             | RX.....   | 2,500               | 11                        | 6                            | 56                           |
|                             | RX.....   | 2,600               | 10.5                      | —                            | —                            |
|                             | RX.....   | 2,800               | 9                         | —                            | —                            |
|                             | RX.....   | 2,900               | 8                         | —                            | —                            |
|                             | RX.....   | 3,220               | 3                         | —                            | —                            |
| Mo-0.5 Ti.....              | SR.....   | 78                  | 125.0                     | 97.0                         | 18                           |
|                             | SR.....   | 1,800               | 83.5                      | 49.0                         | 5                            |
|                             | SR.....   | 2,200               | 45.5                      | 31.0                         | 9                            |
|                             | SR.....   | 2,400               | 22.0                      | 9.0                          | 28                           |
|                             | RX.....   | 2,500               | 17.5                      | 8.5                          | 51                           |
|                             | RX.....   | 2,600               | 15.0                      | 10.0                         | 11                           |
|                             | RX.....   | 2,800               | 10.5                      | 8.0                          | 20                           |
|                             | RX.....   | 3,250               | 5.0                       | —                            | —                            |

It can be seen from this table that the properties of the alloy of the invention are decidedly superior to those of unalloyed molybdenum, particularly at elevated temperatures, and that the alloy of the invention is roughly equivalent to or better than the considerably more expensive arc-cast alloys having 0.5% titanium.

The matrix phase of the alloy of the invention was shown to be homogeneous by anodization techniques known to the art.

The superior properties and economic improvements available through the use of alloys of the invention result in part from: (1) the strengthening of the matrix phase by solid solution hardening due to the addition of tungsten to the molybdenum; (2) the presence of a fine, uniform, insoluble, stable second phase, thoria, which contributes to the high temperature strength and resistance to grain growth at elevated temperatures; and (3) the fact that these two mechanisms interacting provide their beneficial strengthening effects while not destroying the room temperature workability of the alloys. The increases in

the powder-metallurgical alloy structurally consisting of particles of ThO<sub>2</sub> dispersed in a substantially homogeneous tungsten-molybdenum matrix phase.

2. An alloy of claim 1 containing by weight from about 0.1% to about 0.25% ThO<sub>2</sub>, from about 15% to 25% tungsten, balance molybdenum.

3. An alloy of claim 1 containing by weight about 0.2% ThO<sub>2</sub> and about 20% tungsten, the balance being molybdenum.

65

70

## References Cited by the Examiner

A.E.C. bulletin AD-248201, Interim Report No. 5, July 1, 1960-August 31, 1960, Nelson et al., Table V and pp. T34-T36.

BENJAMIN R. PADGETT, Primary Examiner.

REUBEN EPSTEIN, Examiner.

M. J. SCOLNICK, Assistant Examiner.